

Dec. 23, 1958

K. RISCH

2,865,787

PROCESS FOR PRODUCING COLOR EFFECTS ON TEXTILE AND  
OTHER SHEET-LIKE MATERIAL AND PRODUCTS THEREFROM

Filed March 9, 1956



INVENTOR.

KARL RISCH.

BY

Ward, Kiel, Huston, Green & McElhenny,

ATTORNEYS.

## PROCESS FOR PRODUCING COLOR EFFECTS ON TEXTILE AND OTHER SHEET-LIKE MATERIAL AND PRODUCTS THEREFROM

Karl Risch, Wattwil, Switzerland, assignor to Heberlein Patent Corporation, New York, N. Y., a corporation of New York

Application March 9, 1956 Serial No. 570,657

Claims priority, application Germany March 9, 1955

9 Claims. (Cl. 117—71)

This invention relates to a process for producing color effects on textile and other sheet-like material; and products therefrom.

The principal object of the invention is to provide a simple and efficient process for producing novel color effects on the materials mentioned above particularly iridescent effects; and to provide material having such effects.

The invention comprises the novel products as well as the novel processes and steps of processes according to which such products are manufactured, the specific embodiments of which are described hereinafter by way of example and in accordance with which I now prefer to practice the invention.

In carrying out my invention I deposit a metal and metal oxide coating from the vapors thereof on a thin, flexible sheet-like material. Such materials include textile articles such as fabrics, knitted goods, and like textiles, as well as plastic sheets, paper, leather, etc. The plastic sheets may consist of regenerated cellulose, cellulose esters, polyvinyl chloride, polyesters or the like. The metal coats may consist of aluminum, copper, and other metals and the deposition of these coats occurs in a high vacuum. I then deposit on top of said metal deposit, a metal oxide coating from the vapor thereof. Such metal oxide coatings may be tin dioxide, antimony trioxide, cadmium oxide, or lead oxide or the like, and these oxides are vaporized at temperatures of not over about 1500° C. In order to enhance the effects obtained, I may deposit preferably from vapor an organic dyestuff on top of the metal coating and this may be followed by the metal oxide coating. The dyestuff is vaporized at a temperature below that of the vaporization of the metal. The thickness of the metal and metal oxide coatings is such that the flexibility of the resulting textile or other material is not substantially altered. The result is the production of a thin flexible textile or similar material having a metallic lustre and iridescence.

As textiles, I may employ in accordance with my invention, articles of cellulose-containing fiber material such as cotton, viscose rayon, cuprammonium rayon, acetate rayon and furthermore articles of animal fibers such as natural silk or wool and articles of synthetic organic fibers, for instance polyamide fibers (nylon, Perlon), polyester fibers (Dacron, Terylene), polyvinyl-base fibers (Orlon). Furthermore, textile articles consisting of mixtures of the said types of fibers are also suitable. The expression "organic textile material" as used in the appended claims is intended to designate textiles as mentioned above.

As metals to be deposited by vaporization on the sheet-like articles, there are suitable in particular aluminum, copper, tin, silver, gold and other metals which can be vaporized in a high vacuum. It is furthermore possible to deposit different metals one after the other by vaporization onto the same sheet-like articles. It is furthermore advantageous to provide the sheet-like article, be-

fore the treatment with the metal vapor with an embossing effect, for instance a fine rib or Schreiner finish or a glaze friction effect which may be made permanent by means of a synthetic resin. The expression "mechanical effect" as employed in the appended claims is intended to designate an embossing effect such as for instance a fine rib or Schreiner finish or a glaze friction finish, which may be made permanent by means of a synthetic resin.

10 The following examples represent processes which I now prefer to employ in carrying out my invention. It is to be understood that these examples are illustrative and that the invention is not to be considered as restricted thereto except as indicated in the appended claims.

### 15 Example 1

A colored cotton calico is impregnated with an aqueous solution of a melamineformaldehyde precondensate and a catalyst which splits off acid, namely triethanolamine glycolate, calendered on a glazing calender at 180° C. and thereupon cured for 4 minutes at 140° C. The fabric provided in this way with a permanent chintz effect is coated with aluminum by vaporizing the same at a temperature between 800 and 1000° C. in a high vacuum of about  $5 \times 10^{-5}$  mm. mercury. Then the fabric is treated with tin dioxide by vaporizing the same at a temperature between 1000 and 1200° C. in a high vacuum of about  $2 \times 10^{-5}$  mm. mercury. The fabric has a polished metallic lustre and appears reddish or yellow depending on the direction from which it is viewed.

### 30 Example 2

A dyed cotton fabric with 79 ends and picks per inch and the English yarn Number 30 in the warp and the filling is impregnated with the aqueous solution of a melamine-formaldehyde precondensate and an acid-releasing catalyst, namely triethanolamine glycolate, embossed at about 200° C. on a Schreiner calender and thereupon cured for a few minutes at 140 to 160° C. The fabric which is thus imparted a permanent ribbed effect is coated with aluminum as described in Example 1. Then the fabric is coated in a high vacuum of about  $3 \times 10^{-5}$  mm. with antimony trioxide which is vaporized at a temperature of 800 to 1000° C. The fabric has a very attractive metallic lustre and is of different shades depending upon the direction in which it is viewed.

### 35 Example 3

Nylon taffeta is provided on a goffering calender at about 200° C. with a goffered pattern. The fabric is thereupon coated in a high vacuum of about  $5 \times 10^{-5}$  mm. mercury with aluminum which is vaporized at a temperature of 800 to 1000° C., and then with Auramine (tetramethylidiaminobenzophenonimine hydrochloride) which is vaporized at a temperature of 100 to 200° C. Finally the fabric is coated in the same high vacuum with lead oxide which is vaporized at a temperature between 500 and 800° C. The fabric treated in this manner has a goldish yellow metallic lustre, the goldish shade appearing more red or more green depending on whether one looks at the fabric at right angles to its surface or obliquely to same.

### 40 Example 4

A cotton fabric provided with a permanent chintz effect in accordance with Example 1 is first coated with copper by vaporizing the same in a high vacuum of about  $5 \times 10^{-5}$  mm. mercury at a temperature of 1000° to 1100° C. Thereupon the fabric is moated in a high vacuum of about  $3 \times 10^{-5}$  mm. mercury with tin dioxide which is vaporized at a temperature between 1000° and 1200° C. The fabric which has been treated in this manner appears

a deep red or a deep green respectively blue depending on the thickness of the oxide layer applied.

*Example 5*

A plastic sheet consisting of polyethyleneglycolterephthalate is first coated with aluminum as described in Example 1 and thereupon coated in the same high vacuum with fluorescein (phenyloxyfluoren-o-carboxylic acid) which is vaporized at a temperature of 100° to 200° C. Finally the sheet is coated in a high vacuum of  $3 \times 10^{-5}$  mm. mercury with tin dioxide which is vaporized at a temperature between 1000° and 1200° C. The thus treated plastic sheet iridesces in different colors.

The above examples show high resistance to peeling of the coatings from the materials treated.

The iridescent effects obtained by the above examples are due to interference phenomena and the color of the object appears different depending on the thickness and index of refraction of the oxide coating applied. The effects are vivid and interesting.

In the accompanying drawing the figure shows an enlarged diagrammatic perspective of material treated in accordance with the invention.

In the figure, 1 designates a thin sheet-like material having a thin metal coating 2, such as aluminum or other metal deposited thereon, with or without a dye. 3 designates a metal oxide coating deposited on the metal coating 2. The material 1 may be a textile fabric with or without an impregnated resin, or it may be a plastic sheet as above described. The metal oxide coating 3 may be tin dioxide or similar oxide as described above.

I claim:

1. A process, which comprises depositing a metal coating from the vapor thereof on a thin, flexible sheet-like material having a resinous surface adapted to prevent peeling of the metal coating therefrom, and then depositing on top of said metal deposit a metal oxide coating from the vapor thereof, the thickness of said metal and metal oxide coatings being such that the flexibility of the said material is not substantially altered, to produce a sheet-like material having a metallic lustre and iridescence.

2. A process which comprises depositing a metal coating on a thin, flexible sheet-like material having a resinous surface adapted to prevent peeling of the metal coating therefrom by vaporizing the metal in a high vacuum of  $10^{-3}$  to  $10^{-6}$  mm. mercury and then depositing on top of said metal deposit a tin dioxide coating by vaporizing the tin dioxide in the high vacuum, the thickness of said metal and metal oxide coatings being such that the flexibility of the said material is not substantially altered, to produce a sheet-like material having a metallic lustre and iridescence.

3. A process which comprises depositing a metal coating on a thin, flexible sheet-like material having a resinous surface adapted to prevent peeling of the metal coating therefrom by vaporizing the metal in a high vacuum of  $10^{-3}$  to  $10^{-6}$  mm. mercury and then depositing on top of said metal deposit an antimony trioxide coating by vaporization of the antimony trioxide in the high vacuum, the thickness of said metal and metal oxide coatings being such that the flexibility of the said material is not substantially altered, to produce a sheet-like material having a metallic lustre and iridescence.

4. A process which comprises depositing a metal coating on a thin, flexible sheet-like material having a resinous surface adapted to prevent peeling of the metal coating therefrom by vaporizing the metal in a high vacuum of  $10^{-3}$  to  $10^{-6}$  mm. mercury and then depositing on top of said metal deposit a lead oxide coating by vaporizing the lead oxide in the high vacuum, the thickness of said metal and metal oxide coatings being such that the flexibility of the said material is not substantially

altered, to produce a sheet-like material having a metallic lustre and iridescence.

5. A process, which comprises depositing a metal coating from the vapor thereof on a thin, flexible sheet-like material having a resinous surface adapted to prevent peeling of the metal coating therefrom, depositing an organic dye on top of said metal deposit and then depositing on top of said organic dye a metal oxide coating from the vapor thereof, the thickness of said metal and metal oxide coatings being such that the flexibility of the said material is not substantially altered, to produce a sheet-like material having a metallic lustre and iridescence.

6. A process, which comprises depositing a metal coating on an organic textile material having a resinous surface adapted to prevent peeling of the metal coating therefrom and then depositing on top of said metal deposit a metal oxide coating from the vapor thereof, the thickness of said metal and metal oxide coatings being such that the flexibility of the said material is not substantially altered, to produce an organic textile material having a metallic lustre and iridescence.

7. A process which comprises producing a mechanical effect on an organic textile material, depositing a metal coating thereon from the vapor thereof, said material having a resinous surface adapted to prevent peeling of the metal coating therefrom, and then depositing on top of said metal deposit a metal oxide coating from the vapor thereof, the thickness of said metal and metal oxide coatings being such that the flexibility of the said material is not substantially altered, to produce an organic textile material having a metallic lustre and iridescence.

8. A process, which comprises producing a mechanical effect on organic textile material, said mechanical effect being made permanent by means of a synthetic resin, depositing a metal coating thereon from the vapor thereof, said material having a resinous surface adapted to prevent peeling of the metal coating therefrom, and then depositing on top of said metal deposit a metal oxide coating from the vapor thereof, the thickness of said metal and metal oxide coatings being such that the flexibility of the said material is not substantially altered, to produce an organic textile material having a metallic lustre and iridescence.

9. A thin flexible sheet-like material, having a thin metal coating thereon, said material having a resinous surface adapted to prevent peeling of the metal coating therefrom, and above said metal coating, a metal oxide coating, the thickness of said metal and metal oxide coatings being such that the flexibility of the said material is not substantially altered, said material having a metallic lustre and iridescence.

References Cited in the file of this patent

UNITED STATES PATENTS

|    |            |                   |                |
|----|------------|-------------------|----------------|
| 55 | Re. 23,556 | Mochel            | Sept. 30, 1952 |
|    | 1,661,517  | Von Bosse         | Mar. 6, 1928   |
|    | 2,039,372  | Wickman           | May 5, 1936    |
|    | 2,393,640  | King              | Jan. 29, 1946  |
|    | 2,405,662  | McManus et al.    | Aug. 13, 1946  |
|    | 2,422,609  | Auwarter          | June 17, 1947  |
|    | 2,448,511  | Barnes et al.     | Sept. 7, 1948  |
|    | 2,577,957  | Farnsworth et al. | Dec. 11, 1951  |
|    | 2,628,927  | Colbert et al.    | Feb. 17, 1953  |
|    | 2,689,802  | Korver            | Sept. 21, 1954 |
|    | 2,699,402  | Meyer             | Jan. 11, 1955  |
|    | 2,740,732  | Peck et al.       | Apr. 3, 1956   |
|    | 2,748,031  | Kafis             | May 29, 1956   |

FOREIGN PATENTS

|    |         |         |               |
|----|---------|---------|---------------|
| 70 | 179,444 | Germany | Oct. 3, 1906  |
|    | 592,201 | France  | Apr. 25, 1925 |

OTHER REFERENCES

Metal Finishing, July 1949, pp. 42-46, Deposition of  
75 Metallic Films by Vacuum Methods.